

## UNITED STATES PATENT OFFICE

2,071,385

## TREATMENT OF TEXTILE MATERIALS

Edward B. Bell, Lowell, Mass., assignor to The Buromin Company, Pittsburgh, Pa., a corporation of Pennsylvania

No Drawing. Application July 12, 1933,  
Serial No. 680,151

2 Claims. (Cl. 8—5)

The present invention relates to the treatment of textiles and, more particularly, to the dyeing of textiles by the use of dilute solutions of alkali-metal hexametaphosphates.

5 In dyeing, the textile fibers employed are of animal or vegetable origin or of artificial preparation. Examples of the first are wool and silk; of the second, cotton and linen; of the third, "rayon" or other forms of artificial silk made by 10 various processes.

Textile fibers may be dyed between any of the steps used in the manufacture of the finished fabric, namely, they may be dyed in the form of stock, either raw or previously scoured, in the 15 form of partially or fully combed but untwisted fiber, known as sliver or slubbing, in the form of twisted thread or yarn, or finally in the completely woven piece.

When dyed at any of the steps prior to weaving, the object to be attained is the dyeing of the 20 material to an even shade and of the color desired. When dyed in the woven piece, this same end is striven for. On other occasions, however, where the woven piece is composed of 25 threads of different classes of fibers which have different affinities for certain dyes, it is sometimes wished to dye the whole equally and evenly, and at others to choose such dyes or dyeing methods as will color the threads of one composition a 30 certain color and leave the threads of the other material a different color or in their original white condition.

In certain other cases, specific colored designs are given to woven cloth by printing locally thereon 35 certain pigments, dyes or the component parts of dyes and then setting the pigments or developing the dyes of which a certain essential part or parts were locally applied by subjecting the whole piece of cloth to a uniform treatment.

40 For the successful attainment of these desired results, there must be unhindered and even penetration of the dye and its combination with the fiber to be colored.

Penetration or the evenness thereof may be 45 hindered by fats, waxes, oils, or metallic soaps existing either naturally in the fiber or imposed thereon by some process prior to the dyeing operation.

Penetration or the evenness thereof may be 50 hindered by the failure of the dyestuff itself to go into true solution or to assume a sufficiently divided colloidal form in the dye bath. Small traces of extraneous metallic impurities taken up by the dye bath from the metallic walls of the 55 dye kettle or the piping thereto may, in many cases, have most serious results in dulling or otherwise modifying the color produced by the dye. At other times, certain metallic salts are deliberately added to the dye bath or else precipitated on the material to be dyed, either prior 60

to the dyeing thereof or subsequently thereto, for the purpose of firmly fixing the dye to the fiber or for changing the color produced otherwise by the dye alone, to a more desired one.

The following are specific cases of my new 5 method of dyeing. A 30% solution of sodium hexametaphosphate was employed. In some cases, it was adjusted by the addition of small quantities of sodium carbonate and bicarbonate to raise its alkalinity slightly above the neutral 10 point.

A. In attempting to dye rayon slubbing to a deep black, three hundred pounds of the slubbing were loaded into a dyeing machine. The dyeing machine comprised a cylindrical vessel provided with a tight fitting cover. The slubbing was compressed between a perforated top and a perforated bottom in the dyeing vessel and treated with a standard dye liquor having at the beginning of the operation a volume of five hundred 20 gallons. The dye liquor was prepared by dissolving in water:

18 lbs. of the dye known as Direct deep black

E. A. Ex. Color Index 581.

6 lbs. of the dye known as Diazo black B. H. 25 S. W. Color Index 401.

3 lbs. of the pure soap.

1½ lbs. sodium carbonate.

The dyeing vessel had adjacent thereto a smaller vessel open at the top and the two were so interconnected by piping that the dye liquor in the smaller vessel could be forced by a mechanically driven pump, installed in the pipe line leading from the smaller vessel, into the top of the dyeing vessel, through the material to be dyed and returned from the bottom of the dyeing vessel to the smaller auxiliary container. 30 35

The dye liquor could thus be continuously circulated through the material to be dyed.

A small pipe line conveying steam entered the 40 delivery pipe and enabled the circulating dye liquor to be gradually raised to the boiling point. As steam condensed in heating the dye liquor and increased the volume thereof, care was taken to start with only so much liquor as would fill the 45 dyeing vessel and a small part of the auxiliary reservoir, giving room in the balance thereof for the increase in volume of the dye liquor.

The dyeing machine having been prepared as above, the dyeing was started at an approximate 50 temperature of 100 to 110° F. and brought up to the boiling point during a period of thirty minutes. The dye liquor was boiled for twenty minutes. Then, fifteen pounds of sodium sulphate was added and the boiling continued for 55 twenty minutes more. Then, thirty pounds more sodium sulphate was added and the boiling continued for another twenty minutes. Then, sixty pounds more sodium sulphate was added and the boiling continued for another twenty minutes. 60 65

The results of this dyeing attempt were highly unsuccessful. The layer of rayon, perhaps some eight inches in depth, showed but small penetration of dyestuff. It shaded from white at the bottom, through various grays to the wished-for black at the top. The dye seemingly had penetrated scarcely an inch into the material.

Subsequent dyeing attempts were made, using variations in the amounts of sodium carbonate and soap, that were added and further attempts were also made using various preparations reputed to be of value in aiding dye penetration.

I then repeated the dyeing with the dye liquor made as detailed above, except for the addition thereto of 1 1/4 quarts 30% solution of sodium hexametaphosphate. The results were perfectly satisfactory. The rayon at the end of the operation was dyed a uniform deep black.

B. Pieces of woven mixed goods containing besides the main body of wool, certain threads of white silk, were dyed in acid baths in four different ways.

1. In acid dye bath alone.
2. After first mordanting with sodium dichromate.
3. Dyeing and then subsequently mordanting with sodium dichromate.
4. Dyeing with simultaneous addition of sodium dichromate to the dye bath.

Four other pieces of similar goods were then dyed as above, except there was added to the dye bath a dilute solution of sodium hexametaphosphate, i. e., between 1/2 pint and 1 pint of a 30% solution of sodium hexametaphosphate per each 100 gallons of liquor. In the pieces dyed with metaphosphate, the silk threads remained a clearer white than in the pieces dyed without such addition.

C. The addition of an alkali-metal hexametaphosphate improves the process known as cross dyeing, where certain fibers are to be dyed one color and others another color in the same dye bath. Beneficial results in changing the selective affinities of fibers for certain dyes are obtained by the addition to the dye bath of sodium hexametaphosphate.

D. I have found sodium hexametaphosphate to be an assistant in the evenness of dyeing in that process where a dye is first precipitated on the fiber in an acid bath and then its color changed by the subsequent precipitation thereon of a chromium compound by the addition to the bath after the dye is exhausted, of sodium bichromate.

The following dyeing was made: 400 pounds worsted slubbing were dyed in 100 gallons of dye bath made up as follows:

- 8 1/2 lbs. of the dye known as Diamond blue black R. B. N. high conc., new. Color Index 202.
- 1 1/2 lbs. of the dye known as Wool violet 4 B. N. Color Index 698.
- 5/8 lbs. of the dye known as Acid alizarine garnet R. A. Color Index 168.
- 80 lbs. sodium sulphate.
- 25 lbs. 36% acetic acid.

The dye bath containing the material to be dyed was brought to the boil, boiled three-quarters of an hour, 10 pounds 85% formic acid added, boiled one-half hour, 4 1/2 pounds sodium dichromate added and the whole boiled a further half hour.

The dyeing was repeated on a fresh lot of material, the only change being the addition to the

dye bath at the start, of 2 1/2 quarts 30% solution of sodium hexametaphosphate. This resulted in an improved product.

The dye, Diamond blue black R. B. N., dyes red but the subsequent treatment with dichromate turns it to a blue, thus intensifying the black shade of the dye that is present in the largest portion.

Any failure of completeness of the chroming would allow the original red color of the blue black to remain and give a reddish cast to portions of the dyed material. The material dyed without the use of sodium hexametaphosphate not only dyed unevenly, but chromed unevenly as well, whereas the slubbing dyed with the addition of the metaphosphate not only dyed evenly, but chromed more thoroughly and evenly and showed no traces of spots of reddish hue.

E. In order to determine the effect of sodium hexametaphosphate on the deleterious action of small quantities of contaminating metals such as may arise from walls of dyeing vessels, etc. on the colors of delicate shades, I made experimental dyeings in the laboratory in beakers both of glass and Monel metal, putting in some beakers the material to be dyed and the dye bath alone, but in others adding thereto several small pieces of various metals such as iron and brass. I repeated these experiments, changing the procedure in each case only by the addition of a small quantity of sodium hexametaphosphate. I found the metaphosphate had a marked action on the shade-changing effects of the extraneous metallic impurities and, when other well-known mitigating agents were employed, the metaphosphate had a selective action on them.

F. The following is an example of the elimination by sodium hexametaphosphate of the sludge produced on oiled tops when they are dyed and thus obviating a subsequent washing operation:

I dyed 400 pounds worsted slubbing manufactured from oiled tops in 1000 gallons of dye bath made up as follows:

- 12 lbs. of the dye known as Aceko cyanine 3 R. Ex. Color Index 289.
- 1 lb. of the dye known as Wool fast orange G. D. Color Index not listed.
- 1 lb. of the dye known as Diamond flavine G. A. Color Index 110.
- 2 lbs. sodium dichromate.
- 40 lbs. sodium sulphate.
- 7 lbs. 26% ammonia.
- 10 lbs. 56% acetic acid.

This was brought to a boil, boiled one-half hour.

- 2 lbs. acetic acid added and boiled one-half hour.
- 2 lbs. formic acid and then 4 lbs. of the same, with one-quarter hour boiling between them.

An extremely deleterious sludge was found precipitated on the goods. I then repeated this operation on fresh material, but with the addition of 2 1/2 quarts 30% sodium hexametaphosphate. The result was a complete absence of sludge on the goods and enabled the omission of an otherwise necessary washing operation.

The preferred material is the sodium hexametaphosphate known as Graham's salt. If the dihydrogen monosodium orthophosphate is strongly heated, water is driven off and there is an atomic rearrangement within the molecule, whereby sodium acid pyrophosphate is produced.

Upon further heating until melting occurs, more water is driven off, resulting in a further atomic rearrangement, whereby sodium hexametaphosphate is produced.

5 While I prefer to use the sodium hexametaphosphate, other alkali metal hexametaphosphates may be used, such as the potassium and ammonium salts. These alkali-metal hexametaphosphates, appear to have a penetrating action 10 upon the textile fibers, or to assist the penetration of the fibers by the dyestuffs and mordants. They also appear to have a scouring or cleansing action upon the fibers, so that scouring may proceed coincidentally with the dyeing, thus eliminating the expense of a separate scouring step 15 in some instances. The scouring action resulting in removing undesirable substances, is shown

by the elimination of the sludge in one of the examples above.

While I have specifically set forth certain examples showing the practice of my invention, it is to be understood that the invention is not limited thereto, but may be otherwise embodied or practiced within the scope of the following claims. 5

I claim:

1. In the process of dyeing textile materials, the step which consists in subjecting the textiles 10 to a dyeing bath containing an alkali metal hexametaphosphate.

2. In the process of dyeing textile materials, the step which consists in subjecting the textiles 15 to a dyeing bath containing sodium hexametaphosphate.

EDWARD B. BELL.

#### CERTIFICATE OF CORRECTION.

Patent No. 2,071,385.

February 23, 1937.

EDWARD B. BELL.

It is hereby certified that error appears in the printed specification of the above numbered patent requiring correction as follows: Page 2, first column, line 50, for "precipitated" read precipitated; line 56, for the numeral "100" read 1000; and that the said Letters Patent should be read with these corrections therein that the same may conform to the record of the case in the Patent Office.

Signed and sealed this 30th day of March, A.D. 1937.

(Seal)

Henry Van Arsdale  
Acting Commissioner of Patents.

Upon further heating until melting occurs, more water is driven off, resulting in a further atomic rearrangement, whereby sodium hexametaphosphate is produced.

5 While I prefer to use the sodium hexametaphosphate, other alkali metal hexametaphosphates may be used, such as the potassium and ammonium salts. These alkali-metal hexametaphosphates, appear to have a penetrating action 10 upon the textile fibers, or to assist the penetration of the fibers by the dyestuffs and mordants. They also appear to have a scouring or cleansing action upon the fibers, so that scouring may proceed coincidentally with the dyeing, thus eliminating the expense of a separate scouring step 15 in some instances. The scouring action resulting in removing undesirable substances, is shown

by the elimination of the sludge in one of the examples above.

While I have specifically set forth certain examples showing the practice of my invention, it is to be understood that the invention is not limited thereto, but may be otherwise embodied or practiced within the scope of the following claims. 5

I claim:

1. In the process of dyeing textile materials, the step which consists in subjecting the textiles 10 to a dyeing bath containing an alkali metal hexametaphosphate.

2. In the process of dyeing textile materials, the step which consists in subjecting the textiles 15 to a dyeing bath containing sodium hexametaphosphate.

EDWARD B. BELL.

#### CERTIFICATE OF CORRECTION.

Patent No. 2,071,385.

February 23, 1937.

EDWARD B. BELL.

It is hereby certified that error appears in the printed specification of the above numbered patent requiring correction as follows: Page 2, first column, line 50, for "precipitated" read precipitated; line 56, for the numeral "100" read 1000; and that the said Letters Patent should be read with these corrections therein that the same may conform to the record of the case in the Patent Office.

Signed and sealed this 30th day of March, A.D. 1937.

(Seal)

Henry Van Arsdale  
Acting Commissioner of Patents.

CERTIFICATE OF CORRECTION.

Patent No. 2,071,385.

February 23, 1937.

EDWARD B. BELL.

It is hereby certified that error appears in the printed specification of the above numbered patent requiring correction as follows: Page 2, first column, line 50, for "precipitated" read precipitated; line 56, for the numeral "100" read 1000; and that the said Letters Patent should be read with these corrections therein that the same may conform to the record of the case in the Patent Office.

Signed and sealed this 30th day of March, A.D. 1937.

(Seal)

Henry Van Arsdale  
Acting Commissioner of Patents.